

## UNITED STATES PATENT OFFICE

KURT K. LEDIG, OF NEWARK, NEW JERSEY, ASSIGNOR TO AMERICAN PLATINUM WORKS, OF NEWARK, NEW JERSEY, A CORPORATION OF NEW JERSEY

## NIB FOR GOLD PEN-POINTS

No Drawing.

Application filed March 30, 1929. Serial No. 351,464.

This invention relates to nibs especially adapted for use as tips for gold pen points, such nibs usually being made of one or the other metal or a combination of one or the other of the metals of the platinum group (platinum, palladium, iridium, rhodium, ruthenium, osmium) with base metals such as tungsten, tantalum, molybdenum, nickel, cobalt and other suitable metals.

10 Nibs of the class described are usually made from a metal or an alloy which oxidizes rather easily and which has a melting point considerably higher than the metal of the pen point to which it is secured, and in practice great difficulty is experienced in causing complete union of the nib to the pen point during the sweating operation.

In practice it has been found that about 20 out of every 100 gold pens must be discarded 20 because the nibs are not properly united thereto. Obviously such a percentage of loss merits serious consideration, as it materially increases the cost of manufacturing gold pens.

25 This loss is largely due to the fact that when heat is applied to the nib during the sweating operation, it becomes oxidized so that the desired union between the nib and pen point is not obtained.

30 The object of the invention is to provide a method of treating nibs to enable them to be more effectively and expeditiously soldered or otherwise secured to the tips of the gold pen points than has been heretofore possible.

35 This and other objects are accomplished by the novel combination and blending of certain rare or noble metals as hereinafter described and later claimed.

In practicing my invention the nibs are 40 first plated with a suitable metal, it having been found that very satisfactory results are obtained by plating the nibs first with gold, then on top of the gold plate placing a light silver plate.

45 After the nibs have been so plated, they are cleaned in any suitable manner, preferably by washing them in distilled water, after which they are placed in an electric furnace in proximity to a suitable reducing agent, 50 such as charcoal and the temperature of the

furnace is raised to approximately 750 degrees C. or at other temperatures depending upon the plating material employed, the temperature of the furnace being below the melting temperatures of the metals used.

55 The nibs are allowed to remain in the furnace for approximately twenty minutes until the metallic plate has been thoroughly diffused with the metal of the nib, so that an effective alloy is produced.

60 While in the electric furnace under heat, the nibs are protected from oxidation by the reducing agent, the latter also serving to destroy any minute coatings of oxides which may be upon the surfaces of the nibs.

65 It should be noted that other reducing means besides charcoal and the electric furnace may be employed; for example, a diffusion of the plate into the metal of the nib may be accomplished by heating them in hydrogen 70 gas. If plated nibs are already free from oxide when placed into the furnace a diffusion of gold and silver plate into the metal of the nib may be accomplished in a vacuum, or in any inert gas, the essential point being 75 the prevention of oxidation during the heating process.

After a nib has been subjected to heat treatment as set forth above, the gold and silver plates have become diffused with the metal 80 of the nib, the surface of which is now free from oxides and not readily oxidized when heat is thereafter applied. Consequently, when the nib is sweated to a gold pen, no oxides are formed and its surface remains 85 clean so that a positive union between the pen and the nib is obtained.

90 From the above description it will be seen that I have provided an effective method of treating nibs for gold pens so that such nibs may be positively united to gold pens thus eliminating the large waste heretofore common in the manufacture of such gold pens.

Having thus described my invention, what I claim as new and desire to secure by Letter Patent, is:

95 1. A method of treating a nib for a gold pen comprising plating the nib with gold and silver, then heating the plated nib in a furnace containing a reducing material at a tem- 100

perature below the melting points of the metals used.

2. A method of treating nibs for gold pens, consisting of plating the nib with gold and silver, then heating the nib to approximately 750 degrees C. to cause the diffusing of the gold and silver plates with the metal of the nib, the heating being carried on in the presence of a reducing agent to remove and prevent the formation of oxides.

This specification signed this 27th day of March, 1929.

KURT K. LEDIG.

15

20

25

30

35

40

45

50

55

60

65